

April 30, 1935.

B. D. SAKLATWALLA ET AL

1,999,825

TREATMENT OF NELSONITE ORE

Filed Nov. 29, 1932



INVENTORS

Byramji D. Saklatwalla  
Halbert Earl Stibbs  
By their attorney  
Byronia Stibbs, Penelope Blanck

## UNITED STATES PATENT OFFICE

1,999,825

## TREATMENT OF NELSONITE ORE

Byramji D. Saklatwalla and Holbert Earl Dunn,  
Crafton, Pa., assignors to Southern Mineral  
Products Corporation, New York, N. Y., a cor-  
poration of Delaware

Application November 29, 1932, Serial No. 644,833

4 Claims. (Cl. 209—2)

- The present invention relates to the treatment of nelsonite ore, and more particularly to the recovery of ilmenite and apatite concentrates therefrom.
- 5 The term "nelsonite" is applied to ores composed principally of an aggregate of ilmenite and apatite, together with biotite, its related minerals, and clay material in varying proportions. Ilmenite consists essentially of iron and titanium oxides which may be represented generally by the formula  $\text{FeO} \cdot \text{TiO}_2$ . The apatite is a fluorapatite and consists principally of calcium fluorophosphate which may be represented by the formula  $\text{Ca}_5\text{F}(\text{PO}_4)_3$ . Biotite is sometimes designated as black mica or iron-bearing mica because of its iron content. In the nelsonite ore the biotitic mica is in various stages of weathering, some of the mica being in its platy form and some in an altered powder-like condition.
- 10 The principal deposits of nelsonite ore in the United States occur in Nelson and Amherst Counties, Virginia. These deposits have been known for many years and various attempts have been made to work the ores. All attempts to work the ores have heretofore failed because of the seemingly insurmountable difficulty of commercially separating the various constituents of the ore. These extensive nelsonite deposits have therefore heretofore been regarded of little, if any, value.
- 15 We have discovered a process whereby high grade concentrates of ilmenite and of apatite may be recovered from nelsonite ore. The ilmenite concentrate produced is well adapted for the manufacture of titanium dioxide. The apatite concentrate is adapted for conversion into phosphoric acid or phosphoric acid products. The steps of our process are outlined on the accompanying drawing which is a diagrammatic flow sheet. The process will be explained in connection with such flow sheet.
- 20 The nelsonite ore as received in lumps from the mining operations is first put through a rock crusher in which it is crushed, preferably to about 2 inch size. The crushed ore is carried to a storage bin from which it is fed to a grinding mill, preferably a rod mill. The grinding is preferably wet grinding, about 30% by weight of water being added to the material in the rod mill. The rod mill is of the usual construction, the details of which need not be described as they are well-known. The grinding is carried out with steel rods which are preferably light rods about an inch in diameter. The limited amount of water forms a thick mud with the ore being ground. This thick mud tends to cushion the impact of the rods upon each other and to cause the relatively light rods to have a rubbing or scrubbing action upon the particles of the ore rather than an impact crushing action. This is highly desirable since the individual crystals of the ilmenite and apatite should be preserved as such as far as possible, the desirable action of the rod mill being to separate the crystals of ilmenite and apatite from each other and to scrub from such crystals the adhering mica and clay. The rod mill operation is preferably a continuous operation, the crushed rock being fed in at one end and the slurry being discharged from the other end. The degree of particle size reduction is so controlled that while the aggregates consisting of ilmenite and apatite crystals are broken up to free the ilmenite and apatite crystals from each other, the individual crystals are retained as such so far as possible in an uncrushed condition. The softer biotitic alteration products and clays are, however, pulverized to a fine semi-colloidal condition.
- 25 It is important that the degree of crushing of the ore be controlled in order to secure efficient operation in the classification and magnetic separation operations to follow. In order to secure separation of the apatite and ilmenite from each other and from the gangue of the ore, it is necessary to crush to the point where substantially all of the ilmenite and apatite crystals are freed as such from the other materials. It is also important, however, that the separated crystals be retained, so far as practicable, in their original crystalline size in order to secure separation of the crystals from the clay and other fine material in the water classifier and to secure the separation of the ilmenite and apatite crystals from each other and from the undecomposed plate-like biotitic mica in the magnetic separator. We have found that the reduction of the material to retain the crystals of ilmenite and apatite insofar as possible without crushing the individual crystals, gives a crystal size which is well adapted for both the water classification and the magnetic separation.

5

10

15

20

25

30

35

40

45

50

The mud-like slurry from the rod mill is delivered to a vibrating screen of 35 to 48 mesh to the inch. More water is supplied to the screen to assist in the screening operation. All oversize material is returned from the screen to the rod mill.

The nelsonite ore as now obtained from one of the mines in Nelson County, Virginia, contains approximately 43% ilmenite, 20% apatite and 10 37% gangue, consisting of mica alteration products, clay, etc. The screen analysis of the material passing through a 35 mesh screen is approximately as follows:

All pass 35 mesh standard Tyler screen;

|                                    | Percent |
|------------------------------------|---------|
| Retained on 48 mesh                | 3.5     |
| Cumulative retained on 65 mesh     | 13.5    |
| Cumulative retained on 100 mesh    | 28.5    |
| Cumulative retained on 150 mesh    | 38.5    |
| 20 Cumulative retained on 200 mesh | 49.0    |

While 51% passes through 200 mesh.

The slurry which was diluted to about 20% solids by the water added onto the screen, is 25 pumped to a deslimer for the removal of the greater part of the clay and the fine biotite alteration products. These materials are in the class known as slimes and are of a colloidal or semi-colloidal consistency. The deslimer is preferably of the type known as a Calow cone or Allen cone, the constructions of which are well-known in the ore treating art. A deslimer of the cone type consists essentially of a cone-like receptacle of sufficient size to act as a settling tank. 30 The coarser material settles to the bottom of the cone from which it is automatically discharged, while the slimes consisting of the colloidal or semi-colloidal finely divided clays and mica alteration products which constitute the gangue of 35 the ore overflow at the top of the cone. The overflow is run to the dump.

The function of the deslimer is to remove the greater part of the very fine material consisting principally of the colloidal or semi-colloidal clays 40 and biotite alteration products, which would interfere with the most efficient operation of the classifier, to which the material is next conveyed.

The deslimed sand from the deslimer is conveyed to the classifier where more water is added 45 and in which the remainder of the fine material is removed. While it is preferred to secure the removal of the clay material and the biotite alteration products by a two-step separation involving an initial desliming followed by classification, such removal can be secured in a single 50 step in a suitable classifier. However, the commercial classifiers on the market operate much more efficiently if the greater part of the colloidal or semi-colloidal materials are removed by a preliminary desliming operation. Any suitable 55 form of ore classifier may be employed, such as the well-known Akins classifier or the Dorr classifier. The construction and operation of these classifiers is well-known in the ore-treating art and they need not be described in detail. Generally speaking, the classifier, such as the Akins classifier, consists of an inclined trough having a 60 rotating spiral conveyor therein. The material to be classified is run, together with water, into 65 the lower end of the trough which forms a bowl or settling basin. The screw conveyor gently agitates the material and conveys the material from the settling basin or bowl along the inclined trough from which it is discharged. There is a 70 constant overflow from the settling basin, the 75

overflow carrying away the fine material. The sand-like material which is removed by the conveyor is substantially free of all fine material, such as the remaining clay and mica alteration products which were not removed by the deslimer. The sands as they are carried up from the settling basin by the screw conveyor are preferably subjected to water sprays to secure the thorough removal of remaining traces of such fine material.

The classification resulting from the deslimer 10 and classifier should be equivalent to what is known as a free settling period of from 4 to 5½ minutes in order to produce a sand sufficiently clean for magnetic separation and at the same time not to incur too high a loss of apatite 15 mineral in the overflows.

The solid material discharged from the classifier is a fine clean sand which, as obtained from the ore of the mine above mentioned, consists approximately of 69% ilmenite, 21% apatite and 20 10% gangue consisting principally of the platy biotite. The screen analysis of this material is approximately as follows:

|                                           | Percent |
|-------------------------------------------|---------|
| Retained on 35 mesh standard Tyler screen | .2      |
| Cumulative retained on 48 mesh screen     | 25.6    |
| Cumulative retained on 65 mesh screen     | 61.4    |
| Cumulative retained on 100 mesh screen    | 85.0    |
| Cumulative retained on 150 mesh screen    | 93.2    |
| Cumulative retained on 200 mesh screen    | 97.4    |
| Through 200 mesh screen                   | 2.6     |

The clean sand discharged from the classifier is then passed through a drier, which is preferably of the rotary continuous type, which removes the water and delivers dry free flowing sand to a cooler where it is cooled to room temperature. The sand is then passed over a vibrating screen of preferably about 20 meshes to the inch, for the purpose of removing any relatively large particles 40 of foreign matter, such as wood, which may have been accidentally introduced into the material, as well as any large agglomerates produced in the drier. Any traces of clay which may pass the classifier tend to become agglomerated in the drier 45 and are removed by the screen. The over-size refuse from the screen is discarded.

The dry free flowing screened material then passes to a magnetic separator in which there is 50 selective separation of the ilmenite, the apatite and the biotite.

The magnetic separator should be one which secures the selective separation of different constituents of the ore in accordance with their relative magnetic susceptibility. There are various separators on the market which will accomplish this result. The separator is preferably of the well-known induction roll type, the construction of which is well-known in the magnetic separator art and need not be described in detail. In general, it is stated that the magnetic separation is secured by passing the granular sand-like material past a number of rolls. Each roll consists of a series of flat circular soft iron disks with non-magnetic spacers between them. An electromagnet is located in proximity to the face of the roll and the material passes between the roll and the magnet face. The spacing apart 60 of the soft iron disks of the roll serves to concentrate the magnetic field toward these disks, so that the magnetizable particles of the material are attracted to the roll and are carried around 65 for removal at a magnetically neutral point of the roll. In the induction roll type of machine 70 which we have employed there are six induction 75

rolls. The magnetic force exerted by the various rolls is progressively increased from the first to the last roll, the first roll being relatively weakly magnetic.

5 The ilmenite which has a magnetic attractive force of about 25 as compared with 100 for iron particles, is separated out by the first three rolls. The magnetic effect of these rolls, while strong enough to remove the strongly magnetic ilmenite, 10 is not strong enough to remove the biotite which has a magnetic attractive force of about 3, and the apatite which has a magnetic force of about 0.2, as compared with 100 for iron particles. The last three rolls, which are more strongly magnetized 15 than the first three, separate the weakly magnetic biotite from the apatite.

The material separated by each roll is run into bins and the apatite, which is substantially non-magnetic, passes through the machine and is run 20 into an apatite storage bin. The biotite, which is a waste product, is discarded. Under properly controlled conditions it is possible to secure a recovery of from 90 to 95% of the ilmenite content of the ore and to secure a recovery of from 25 70 to 75% of the apatite content of the ore. The reason for the greater percentage of the ilmenite recovery is that the ilmenite crystals are harder and there is less loss of ilmenite in the desliming and classifying operations than there is of 30 the softer apatite. The ilmenite fraction is a high-grade concentrate containing about 95 to 96% of ilmenite. This concentrate is sufficiently pure to furnish a good raw material for the production of titanium dioxide according to the 35 usual methods of preparing titanium dioxide from ilmenite. The apatite fraction is also a high-grade concentrate containing about 97% or over of apatite. In case the ore is treated for the recovery of the ilmenite fraction only, there will 40 be no separation of the biotite from the apatite and both will be discarded together.

While we have specifically described the preferred procedure in practicing our invention, it is to be understood that the invention is not limited 45 to its preferred embodiment, but may be otherwise embodied and practiced within the scope of the following claims.

We claim:

1. The process of recovering ilmenite and apatite concentrates from nelsonite ore, which comprises adding about 30% of moisture to the ore and subjecting the ore together with its clay constituents to impact of steel rods in a rod mill to a limited extent sufficient to reduce the gangue but not to pulverize the ilmenite and apatite crystals, separating the finely divided gangue from the ilmenite and apatite, and thereafter magnetically selectively separating the ilmenite, 10 apatite and biotite. 5

2. The process of recovering ilmenite and apatite concentrates from nelsonite ore, which comprises adding about 30% of moisture to the ore and subjecting the ore together with its clay constituents to impact of steel rods in a rod mill to a limited extent sufficient to reduce the gangue but not to pulverize the ilmenite and apatite crystals, subjecting the ore to a water classification to separate the finely divided gangue from 15 the ilmenite and apatite, and thereafter magnetically selectively separating the ilmenite, apatite and biotite. 20

3. The process of recovering ilmenite and apatite concentrates from nelsonite ore, which comprises adding about 30% of moisture to the ore and subjecting the ore together with its clay constituents to impact of steel rods in a rod mill to a limited extent sufficient to reduce the gangue but not to pulverize the ilmenite and apatite 25 crystals, separating the finely divided gangue from the ilmenite and apatite, and thereafter magnetically separating the ilmenite from the apatite and biotite. 30

4. The process of recovering ilmenite and apatite concentrates from nelsonite ore, which comprises adding to the ore sufficient water to produce a thick mud when ground, and subjecting the ore together with its clay constituents to impact of steel rods in a rod mill to a limited extent sufficient to reduce the gangue but not to pulverize the ilmenite and apatite crystals, separating the finely divided gangue from the ilmenite and apatite, and thereafter magnetically selectively separating the ilmenite, apatite and biotite. 40 45

BYRAMJI D. SAKLATWALLA.  
HOLBERT EARL DUNN.